

April 24, 1962

T. R. A. DAVEY

3,031,296

SEPARATION OF LEAD AND ZINC

Filed Oct. 13, 1958



Fig. 1.



Fig. 2.



Fig. 3.

Thomas Ronald Albert Davey  
Inventor  
by  
Pennie, Edmonds, Morton, Barrows & Taylor

1

3,031,296

## SEPARATION OF LEAD AND ZINC

Thomas Ronald Albert Davey, Avenmouth, England, assignor to Metallurgical Processes Limited, Nassau, Bahamas, and The National Smelting Company Limited, London, England, carrying on business together in the Bahamas under the name and style of Metallurgical Development Company

Filed Oct. 13, 1958, Ser. No. 766,785

Claims priority, application Great Britain Oct. 18, 1957  
4 Claims. (Cl. 75—88)

This invention relates to the separation of lead and zinc from mixtures thereof.

A continuous process is known for removing zinc from lead by vacuum distillation, which produces metallic zinc containing a little lead from lead which has been desilverized by treatment with zinc. The zinc produced by this distillation is designed for re-use in the desilverizing of further lead bullion. In this process, zinciferous lead is distilled in a vacuum chamber to produce zinc vapour which condenses on a core of solid zinc and runs down into a collecting pool. The lead content of this metallic zinc is sufficiently high to restrict the number of commercial purposes to which it can be put.

It is known that zinc of low lead content can be produced from lead-containing zinc by a process of distillation with refluxing at atmospheric pressure. In a known process, the impure zinc is volatilized and the vapour is passed through a refluxing column containing a large number (generally greater than twenty) of trays for condensation and re-evaporation, and zinc that is substantially free from lead is condensed from the vapour leaving the top of the refluxing column.

The present invention consists of a method of separating pure zinc from zinc of low lead content in which the lead-containing zinc is distilled under vacuum at temperatures of about 450° to 500° C., whereby the vapour obtained is practically free from lead. Under vacuum therefore the zinc (containing about 1% lead) can be distilled, and without the use of any refluxing column, zinc that is substantially free from lead can be obtained by condensing the zinc vapour so produced.

The present invention further consists of a process in which zinc-containing lead is distilled under vacuum and the lead contaminated zinc vapour is condensed in a circulated stream of molten zinc, which is at a lower temperature than the zinc-containing lead, zinc vapour being simultaneously evaporated from the circulated stream of molten zinc and condensed in a zone that is at a lower temperature than the circulated stream of molten zinc.

In one form of the present invention, zinc-containing lead, at a temperature above the melting point of zinc, flows through an outer annular evaporation zone of an evacuated vessel, a stream of molten lead-containing zinc at a lower temperature and still above the melting point of zinc, is circulated through an intermediate annular zinc-vapor refining zone of the evacuated vessel, and centrally disposed cooling means are provided in an innermost annular condensation zone of the evacuated vessel. By this means some of the zinc is evaporated from the zinc-containing lead, and is condensed in the stream of molten zinc and condensed in a zone that is at a lower zone. Zinc vapour is simultaneously evaporated from the stream of molten lead-containing zinc on the inner sides of the intermediate annular zone and solid zinc condenses and accumulates on the cooling zone to a point at which its temperature rises to the melting point of zinc and thereafter the zinc condensed here runs off as molten zinc, the amount of molten zinc thus condensed being approximately equal to the amount of zinc evaporated from the zinc-containing lead. The circulated stream of molten lead-containing zinc is maintained at a temperature higher

2

than the melting point of zinc but lower than that of the zinc-containing lead, and lead accumulates in this lead-containing zinc until it becomes saturated with lead, and zinc-saturated lead separates from a zone of the circulation system outside the evacuated vessel.

The invention will be further described with reference to the accompanying drawing.

FIGURE 1 is a sectional elevation of one form of distillation apparatus incorporating the improvement.

FIGURE 2 is a section on the line II—II of FIGURE 1 and,

FIGURE 3 is an enlarged detail of FIGURE 1.

Lead containing about 1% zinc is supplied to the chamber 1 through a pipe 2 situated just below the surface of the molten lead in the annular well 3 at a temperature of about 560° C. The lead in this well builds up behind a rectangular flange 4 welded to the top of an outer annular spreading wall 5. This flange has holes 6 through which lead seeps evenly around the perimeter of the spreading wall 5. This wall has an outwardly divergent lip 7 over which the lead flows in a thin stream "coating" the inside of the wall 5 with a layer of lead. The evaporating conditions in the chamber, with a pressure of less than 10 mm. mercury, cause the zinc in this lead to progressively evaporate out into the outer zone 8 of the chamber, as the lead flows down the wall 5 into a trough 9, at the bottom of which a pipe 10 leads to a bath of lead in the pot 11 from which it runs continuously or can be tapped from time to time; the length of the pipe 10 above the lead in pot 11 is greater than the height of a barometric column of lead. The zinc vapour passes inwards towards an intermediate annular system of inclined shelves one above the other, which face alternately outwards 12 and inwards 13 with connecting rods 12a and 13a (FIGURE 3). These shelves may be constructed of refractory material or enamelled steel resistant to corrosion by zinc. These shelves are supplied with a continuous stream of molten zinc at a temperature of about 450° to 500° C. After circulating over the shelves the molten zinc falls into an annular trough 14a connected by a pipe 14b to a bath 14, from which a pump 15 sends it up the pipe 16 and into an annular trough 17, from which it overflows to cascade over the shelves again. The lead which is collected by the zinc separates out of the zinc in the bath 14 and can be taken off at 18.

The surfaces of the outwardly facing shelves 12, over which the zinc is flowing, are exposed to the incoming zinc vapor, containing less than 1% lead, coming from the relatively hot zinc vapor in zone 8, so that the zinc vapor condenses on shelves 12, and the latent heat of condensation of this zinc causes the temperature of the liquid zinc to rise by between 5° C. and 50° C. From each of the shelves 12, the liquid zinc then flows on to one of the inwardly facing shelves 13, and, owing to the lower pressure of zinc vapor prevailing in the inner zone 19, the zinc re-evaporates from shelves 13, the latent heat of evaporation thus abstracted causing the temperature of the liquid zinc flowing over these shelves 13 to fall by approximately the same amount as it rose over shelves 12. This re-evaporated zinc vapor contains only 0.01% or less lead. The lower zinc pressure in zone 19 prevails because the zinc vapor condenses on the zinc collar 20. This vapour condenses on the innermost zinc collar 20 which builds up during the course of the process as a solid deposit on the condenser 21 with cooling pipe 21a until the temperature on the outside is sufficient to cause the zinc to remain liquid and drip down off the collar. The molten condensed zinc flows down pipe 25, the lower end of which is submerged in molten zinc contained in pot 26, the length of pipe 25 being greater than the height of a barometric column of zinc. Any zinc

vapour which enters the condenser 21 is prevented from forming a solid deposit by the installation of a radiant heater 22. The cold trap 23 is removable in order to clean out any deposit which may form on its water cooled walls. No zinc must be allowed to build up in the vacuum pipe 24.

Various modifications may be made within the scope of the invention.

I claim:

1. In the process for separating and recovering zinc from lead of low zinc content in which molten zinc-containing lead at a temperature above the melting point of zinc is introduced under vacuum into an evaporation zone to evaporate therefrom zinc vapors containing a small quantity of lead, and in which these lead-contaminated zinc vapors are condensed to liquid metal on a body of solidified zinc in a condensation zone maintained at a lower temperature than that of the evaporation zone, the liquid metal condensate being collected and recovered, the improvement which comprises the provision of an intermediate zinc-vapor refining zone disposed between said evaporation and condensation zones, said zinc-vapor refining zone having a circulating stream of molten zinc flowing therethrough at a temperature between that of the evaporation zone and that of the condensation zone, the lead-contaminated zinc vapors from the evaporation zone condensing in the circulating stream of molten zinc and zinc vapor contaminated with a lesser amount of lead simultaneously evaporating from said circulating stream of molten zinc without supplying additional heat to the intermediate zinc-vapor refining zone, the zinc vapor evaporated from the refining zone being condensed to relatively pure liquid zinc metal on the body of solidified zinc in the condensation zone.

2. In apparatus for separating zinc from lead of low zinc content comprising an evacuated vessel within which is provided an outermost annular spreading tube over

which the molten zinc-containing lead flows in an even layer at a temperature above the melting point of zinc, and an innermost centrally disposed cooling means on which zinc vapors evaporated at the spreading tube are condensed, the improvement which comprises the provision of an intermediate annular zinc-vapor refining means disposed between said outermost spreading tube and said centrally disposed cooling means, said zinc-vapor refining means comprising a system of inclined trays disposed one above the other and facing alternately outwards and inwards, and means for maintaining a flow of molten zinc over said trays at a temperature above the melting point of zinc but below the temperature of the molten zinc-containing lead flowing over the spreading tube.

3. Apparatus according to claim 2 having collecting means for collecting molten zinc running off from the surface of solidified zinc condensed on the centrally disposed cooling means.

4. Apparatus according to claim 2 having collecting means for collecting lead-containing molten zinc that runs off the lower end of the annular zinc-vapor refining means, and means outside the evacuated vessel for recovering zinc-saturated lead which separates from said lead-containing zinc.

References Cited in the file of this patent

UNITED STATES PATENTS

|           |              |       |               |
|-----------|--------------|-------|---------------|
| 2,312,811 | Gentil       | ----- | Mar. 2, 1943  |
| 2,349,409 | Davis        | ----- | May 23, 1944  |
| 2,478,594 | Queneau      | ----- | Aug. 9, 1949  |
| 2,720,456 | Davey        | ----- | Oct. 11, 1955 |
| 2,823,111 | Davey et al. | ----- | Feb. 11, 1958 |
| 2,939,783 | Lundevall    | ----- | June 7, 1960  |

FOREIGN PATENTS

|         |               |       |               |
|---------|---------------|-------|---------------|
| 711,954 | Great Britain | ----- | July 14, 1954 |
|---------|---------------|-------|---------------|

UNITED STATES PATENT OFFICE  
CERTIFICATE OF CORRECTION

Patent No. 3,031,296

April 24, 1962

Thomas Ronald Albert Davey

It is hereby certified that error appears in the above numbered patent requiring correction and that the said Letters Patent should read as corrected below.

Column 1, lines 62 and 63, for "molten zinc and condensed in a zone that is at a lower zone" read -- molten lead-containing zinc in the intermediate annular zone --.

Signed and sealed this 14th day of August 1962.

(SEAL)

Attest:

ERNEST W. SWIDER  
Attesting Officer

DAVID L. LADD  
Commissioner of Patents